

# United States Patent Office

3,154,614

Patented Oct. 27, 1964

1

3,154,614

## PROCESS FOR SPINNING A HIGH VISCOSITY, HIGH GAMMA VISCOSITY

Yoshikazu Aoki, Otsu, and Teruji Kamei, Sakyo-ku, Kyoto, Japan, assignors to Tachikawa Research Institute, Higashiyama-ku, Kyoto, Japan, a corporation of Japan  
No Drawing. Filed June 27, 1962, Ser. No. 205,565  
5 Claims. (Cl. 264—188)

This invention relates to a process for producing rayon as regenerated cellulose in the form of filaments or fibers. In particular, it is concerned with an improved method for regenerating cellulose by the spinning of viscose in the manufacture of viscose rayon yarn. This is a continuation-in-part of application Serial No. 64,730, now abandoned, filed October 25, 1960.

The basic process contemplated by this invention essentially entails the spinning of unripened viscose in a low acid concentration bath, the temperature of the bath being controlled and the viscose having a high degree of polymerization. Processes of this type are known to the art being described, for example, in U.S. Patents Nos. 2,592,355, 2,732,279 and 2,607,955. These processes have proved dissatisfactory from the standpoint that the spinning velocity may not be increased beyond a certain limit without seriously diminishing the tenacity of the resulting filament or fiber and jeopardizing the stability of the process itself due to actual breakage of the semi-coagulated viscose thread within the bath or outside thereof as it is being reeled onto the stretching or tension imparting components. Thus far, it has been found that for high viscosity viscose a spinning velocity of 20 meters per minute is about the permissible maximum in commercial practice and this relatively low velocity has been considered a disadvantage.

The inventive concept herein is directed toward the solution of the problem of spinning viscose which has a high degree of polymerization. That the problem is significant is due to the fact that the higher the degree of polymerization of the spun fiber, the more nearly will it have the intrinsic properties of natural fiber. As pointed out in Patent No. 2,732,279, it had been thought that an essential condition of spinning high D.P. viscose is to keep the bath temperature below 30° C. This requirement was due to the unduly high rate of regeneration of the viscose rayon fiber at higher temperatures which adversely affected the strength of the regenerating filaments. However, the relatively low bath temperature limits the permissible spinning velocity. According to the instant process, the high D.P. viscose is spun in a coagulating bath the temperature of which is raised above 30° C. which, as is well known, enables higher spinning velocities. Concomitantly, however, the nature and percentage composition of the bath is maintained within critical limits and also in critical relation to the temperature so as to permit the raised temperature without the resulting adverse effect thereof.

The present invention envisions, therefore, a spinning process in which high D.P. viscose is spun at 30 meters per minute or more and which is adapted to produce filaments or fibers with superior properties. The sulphuric acid concentration in the bath is low, for example, within the range of 1 to 30 grams per liter and the initial material is unripened viscose having a high viscosity or degree of polymerization. A weak acid bath is hereby defined as one in which the acid concentration is within the approximate limits stated above and high viscosity cellulose has a viscosity above 250. In addition, the gamma value of the viscose is above 50 and preferably between 50 and 100. Principal features of the inven-

2

tion relate to such factors as temperature of the spinning bath and zinc sulphate concentration and are directly productive of the desired higher spinning velocity and stability of the spinning process as an operation as well as improvement in the characteristics of the resulting fibers. In order for these improvements to be obtained, it is required that the temperature of the spinning bath be not less than 30° centigrade and the  $ZnSO_4$  concentration be within the range of from 0.2 to 2.0 grams per liter. Moreover, it was found that permissible spinning velocity and bath temperature over 30° centigrade can be directly related provided the bath contains the necessary controlled amount of  $ZnSO_4$ . In conventional processes which do not provide  $ZnSO_4$  in the bath the regeneration of the viscose rayon fiber proceeds so rapidly that its strength is not sufficient to withstand the friction from movement of the spinning liquor at the higher spinning velocities. This is due to the fact that the thread cannot be sufficiently stretched when regeneration occurs rapidly. It is the function of the  $ZnSO_4$  in controlled amounts to slow the regeneration process or the decomposition of the viscose as measured by its  $\gamma$ -value so that stretching can occur smoothly and as long as regeneration occurs. The stretching may be effected by means of special godets such as are described and illustrated in U.S. Patent No. 2,732,279. As the condition of the viscose changes from a  $\gamma$ -value to say 30 to a state where the viscose has completely decomposed and its  $\gamma$ -value is, therefore, 0, a substantial amount of stretching is possible either inside or outside the bath provided the change in state of the material is controlled which is the function of the  $ZnSO_4$ . Under these stipulated conditions, the thread can, in fact, be stretched more than 200% which will assure sufficient tenacity of the coagulating fiber to allow a marked increase in spinning velocity.

The following relation between temperature of the spinning bath and concentration of  $ZnSO_4$ , which are the key factors in the improved spinning process, and spinning velocity have been observed.

| Temperature of the spinning bath—centigrade | Concentration of $ZnSO_4$ , Grams per Liter | Favorable Spinning Velocity, Meters per Minute |
|---------------------------------------------|---------------------------------------------|------------------------------------------------|
| 30°-35°                                     | 0.2-0.5                                     | 35                                             |
| 35°-40°                                     | 0.5-0.7                                     | 40                                             |
| 40°-50°                                     | 0.7-2.0                                     | 50                                             |

The filaments obtained by this process have a homogeneous distribution of the zinc xanthate throughout the viscose column being incorporated therein under high osmotic pressure. The fibrous material thus formed is very strong. In addition, the resulting fiber is round in cross section, superior in dyestuff absorption, is low swelling in water and dilute alkali solution and has a high wet modulus.

The following examples may help to give a clearer understanding of our process for producing rayon which includes, in particular, the improved method of viscose spinning.

### Example 1

Wood pulp with a degree of polymerization of 850 is steeped one hour at 20° centigrade in 18% NaOH solution, and after being pressed to 2.6 times the weight of the original pulp, it is crushed at 18° centigrade for 2 hours. Alkali-cellulose without aging, is subjected to xanthation with 45%  $CS_2$  to the weight of the cellulose at 19-28° centigrade for 2.5 hours. The composition of the resulting viscous is 5% cellulose and 3.5% NaOH. This viscose is filtered, deaerated and spun as soon as

possible after xanthation, its viscosity (by falling ball method) being 250 and its  $\gamma$ -value 60. The spinning conditions are as follows:  $H_2SO_4$  concentration in the spinning bath is 8.0 grams per liter,  $ZnSO_4$  concentration in the bath is 0.5 gram per liter, temperature of the bath is 35° centigrade, and the thread is stretched to 210% by a godet located outside of the bath, and the final spinning velocity is 40 meters per minute. Characteristics of filament are: 1.4 denier, dry tenacity 4.3 grams per denier, wet tenacity 3.2 grams per denier, dry elongation 12.7%, wet elongation 13.5%, dry knot tenacity 2.1 grams per denier, flex cycle 650.

*Example 2*

Linter pulp with degree of polymerization of 1650 is steeped in 19% NaOH solution for 2 hours at 20° centigrade and after being pressed to 2.8 times of the weight of pulp, it is disintegrated for 2.5 hours at 31° centigrade. Without aging, the alkali-cellulose is xanthated with  $CS_2$  in the amount of 60% to the weight of the cellulose for 3 hours at 20-33° centigrade. The composition of the viscose thus obtained is 4.5% cellulose and 4.5% NaOH, its viscosity being 450 and its  $\gamma$ -value 80. The spinning is carried out in a spinning bath containing 5.4 grams per liter  $H_2SO_4$ , 1.0 gram per liter  $ZnSO_4$  and at a bath temperature of 40° centigrade. The spinning velocity is 45 meters per minute. The thread, after traveling 15 cm. in the bath, is stretched to 250% by a godet immersed in the spinning bath. The characteristics of the resulting fiber are: 1.0 denier, dry tenacity 5.5 grams per denier, wet tenacity 4.2 grams per denier, dry elongation 12.4%, wet elongation 16.5%, dry knot tenacity 2.4 grams per denier, flex cycle 1100.

*Example 3*

Wood pulp with a degree of polymerization of 1270 is steeped for 2 hours at 20° C. in 19.0% NaOH solution, and after being pressed 2.8 times the weight of the original pulp, it is crushed at 24° C. for 2 hours. Alkali-cellulose, thus obtained, is subjected to xanthation with 55%  $CS_2$  to the weight of the cellulose at 20-28° C. for 2.5 hours. The composition of the resulting viscose is 4.5% cellulose and 3.8% NaOH. After being filtered and deaerated, this viscose is spun, its viscosity (by falling ball method) being 750 and its  $\gamma$ -value 100. The spinning conditions are as follows:  $H_2SO_4$  concentration in the spinning bath is 9.2 grams per liter,  $ZnSO_4$  concentration in the bath is 0.2 gram per liter, temperature of the bath is 30° C., and the thread of 1,000 filaments is stretched by a godet, and the final velocity is 35 meters per minute.

The characteristics of the resulting fibers are: 1.2 denier, dry tenacity 5 grams per denier, wet tenacity 4 grams per denier, dry elongation 13%, wet elongation 16%, dry knot tenacity 2.1 grams per denier.

*Example 4*

Wood pulp with a degree of polymerization of 1,100 is steeped for 2 hours at 20° C. in 18.5% NaOH solution, and after being pressed 2.8 times the weight of the original pulp, it is crushed at 27° C. for 2.5 hours, alkali-cellulose, thus obtained, is subjected to xanthation with 50%  $CS_2$  to the weight of the cellulose at 19-27° C. for 2.5 hours. The composition of the resulting viscose is 5.2% cellulose and 3.6% NaOH. After being filtered and reaerated, this viscose is spun, its viscosity being 610 and its  $\gamma$ -value 85. The spinning conditions are as follows:  $H_2SO_4$  concentration in the spinning bath is 15.6 grams per liter,  $ZnSO_4$  concentration in the bath is 0.5 gram per liter, temperature of the bath is 35° C., and the thread of 6,000 filaments is stretched by a godet, and the final spinning velocity is 40 meters per minute.

The characteristics of the resulting fibers are: 1.5 denier, dry tenacity 4.8 grams per denier, wet tenacity 3.6 grams per denier, dry elongation 12%, wet elongation 15%, dry knot tenacity 1.8 grams per denier.

*Example 5*

Wood pulp with a degree of polymerization of 950 is steeped for 2 hours at 20° C. in 18.2% NaOH solution, and after being pressed 2.9 times the weight of the original pulp, it is crushed at 28° C. for 2.5 hours, alkali-cellulose, thus obtained, is subjected to xanthation with 45%  $CS_2$  to the weight of the cellulose at 18-26° C. for 2.5 hours. The composition of the resulting viscose is 5.5% cellulose and 3.3% NaOH. After being filtered and deaerated, this viscose is spun, its viscosity being 520 and its  $\gamma$ -value 75. The spinning conditions are as follows:  $H_2SO_4$  concentration in the spinning bath is 30.0 grams per liter,  $ZnSO_4$  concentration in the bath is 1.2 grams per liter, temperature of the bath is 50° C., and the thread of 18,000 filaments is stretched by a godet, and the final spinning velocity is 50 meters per minute.

The characteristics of the resulting fibers are: 1.5 denier, dry tenacity 4.5 grams per denier, wet tenacity 3.2 grams per denier, dry elongation 11%, wet elongation 14%, dry knot tenacity 1.6 grams per denier.

As mentioned above, the complete absence of the  $ZnSO_4$  in the spinning bath precludes the possibility of imparting sufficient stretch to the coagulating material to permit of high velocity spinning. On the other hand too much  $ZnSO_4$  in the bath which has a low acid concentration and low temperature causes the formation of the zinc xanthate to become too irregular which also results in the formation of a thread of low tenacity which cannot be spun with higher than conventional spinning velocities.

Various modifications in the process as above described may be effected by persons skilled in the art without departing from the principle and scope of invention as defined in the appended claims.

What is claimed is:

1. In the process for the manufacture of rayon filament or fiber in a weak sulphuric acid bath from viscose, the steps of extruding unripe viscose having a gamma value above 50 into the bath having a  $ZnSO_4$  concentration which varies with the temperature of the bath from 0.2 gram per liter  $ZnSO_4$  concentration for a temperature of 30° centigrade to 2.0 grams per liter  $ZnSO_4$  concentration for a temperature of 50° centigrade.
2. In the process for the manufacture of rayon filament or fiber in a weak acid bath from viscose, the steps of extruding unripe viscose having a gamma value above 50 into the bath having a sulphuric acid concentration of from approximately 1 to 30 grams per liter and a  $ZnSO_4$  concentration which varies with the temperature of the bath from 0.2 gram per liter  $ZnSO_4$  concentration for a temperature of 30° centigrade to 2.0 grams per liter  $ZnSO_4$  concentration for a temperature of 50° centigrade.
3. In the process for the manufacture of rayon filament or fiber in a weak sulphuric acid bath from viscose, the steps of extruding unripe viscose having a gamma value above 50 into the bath having a  $ZnSO_4$  concentration which varies with the temperature of the bath from 0.2 to 0.5 gram per liter  $ZnSO_4$  for a temperature of 30° centigrade, to 0.4 to 0.7 gram per liter  $ZnSO_4$  for a temperature range of 35° to 40° centigrade, to 0.5 to 2.0 grams per liter  $ZnSO_4$  for a temperature of 50° centigrade.
4. In the process for the manufacture of rayon filament or fiber in a weak acid bath from viscose, the steps of extruding viscose having a viscosity above 250 and a gamma value above 50 into the bath having a sulphuric acid concentration of from approximately 1 to 30 grams per liter and a  $ZnSO_4$  concentration which varies with the temperature of the bath from 0.2 to 0.5 gram per liter  $ZnSO_4$  for a temperature of 30° centigrade, to 0.4 to 0.7 gram per liter  $ZnSO_4$  for a temperature range of 35° to 40° centigrade, to 0.5 to 2.0 grams per liter  $ZnSO_4$  for a temperature of 50° centigrade.

5. In the process for the manufacture of rayon filament or fiber in a weak acid bath from viscose, the steps of extruding viscose having a viscosity above 250 and a gamma value above 50 into the bath having a sulphuric acid concentration of from approximately 1 to 30 grams per liter, a  $ZnSO_4$  concentration which varies with the temperature of the bath from 0.2 to 0.5 gram per liter  $ZnSO_4$  for a temperature of 30° centigrade, to 0.4 to 0.7 gram per liter  $ZnSO_4$  for a temperature range of 35° to 40° centigrade, to 0.5 to 2.0 grams per liter  $ZnSO_4$  for a temperature of 50° centigrade, the permissible spinning velocity being 35 meters per minute at 30° centigrade, to 40 meters per minute at 35° to 40° centigrade, to 50 meters per minute at 50° centigrade.

10

## References Cited in the file of this patent

## UNITED STATES PATENTS

|           |           |        |                |              |
|-----------|-----------|--------|----------------|--------------|
| 2,307,864 | 1/43      | Soukup | -----          | 264—188      |
| 5         | 2,607,955 | 8/52   | Drische et al. | -----264—181 |

## OTHER REFERENCES

1954, Cellulose and Cellulose Derivatives, Part II, edited by Ott et al., 2nd edition, published by Interscience Publishers, Inc., New York.

ALEXANDER H. BRODMERKEL, *Primary Examiner.*  
MICHAEL V. BRINIDISI, MORRIS LIEBMAN,  
*Examiners.*